

Dec. 8, 1964

R. A. ALLIEGRO

3,160,480

REFRACTORY ARTICLES BONDED TO A METAL BASE

Filed May 11, 1961

*Fig. 1.*



*Fig. 2.*



*Fig. 3.*



INVENTOR

RICHARD A. ALLIEGRO

BY

*Richard Alliegro*  
ATTORNEY

1

3,160,480  
REFRACTORY ARTICLES BONDED TO A  
METAL BASERichard A. Aliegro, Holden, Mass., assignor to Norton  
Company, Worcester, Mass., a corporation of  
MassachusettsFiled May 11, 1961, Ser. No. 109,432  
3 Claims. (Cl. 29—195)

This invention relates to the bonding of refractory articles to supporting metallic bases and to the composite and integral articles thereby produced. More particularly, this invention relates to a method of bonding refractory articles formed from borides or carbides to bases of iron, steel, or other conductive metals to provide composite articles wherein the desirable characteristics of the refractory material may be conveniently utilized.

The application of refractories such as borides and carbides in various industrial processes is becoming more and more prevalent. Such materials as titanium diboride, zirconium diboride and titanium carbide, for example, when used as cathodes in electrolytic cells, have shown distinct advantages over the standard iron cathode conventionally utilized. One specific application is the use of these materials in cells for the reduction of alumina to aluminum metal.

Titanium diboride, for example, when fabricated to certain specifications, is characterized by a high density (above 88 percent of its theoretical value), low electrical resistivity (less than 30 micro-ohm centimeters), high strength (greater than 40,000 p.s.i. cross bending at room temperature), low solubility in molten aluminum and excellent resistance to the electrolytes such as cryolite used in aluminum cells. Zirconium diboride and titanium carbide exhibit similar properties.

One major problem associated with the use of these materials is the cost of the materials themselves both in powder form and in fabricated shapes. The production of borides and carbides of high purity is expensive and fabrication into shapes necessitates the use of great degrees of heat and pressure because of the relative refractoriness of these materials. Cathodes for electrolytic cells are produced in the form of bars and range in size from about 2 to 8 inches in diameter and from about 18 to 24 inches in length while the "working end" or tip portion actually in contact with the aluminum is only about 2 to 4 inches of this length. The remainder of the bar extends from the working end and is connected to a source of electrical power.

It has been found that a considerable saving of expense in the production of cathodes may be achieved if only the tip or that portion in or adjacent the electrolyte bath is formed of the costly refractory and the remainder formed of a cheaper metal such as iron or steel. However, the direct bonding of metal to the tip such as by welding has been found to be impractical largely due to the great difference in coefficients of expansion of these materials. Titanium diboride, for example, has a coefficient of expansion of  $8.1 \times 10^{-6}$  over the temperature range of 20° to 800° C., while iron or steel has an average coefficient of expansion of about  $14 \times 10^{-6}$  over the temperature range of 20° to 700° C. Furthermore, the refractories such as titanium diboride lack ductility. Therefore, the expansion and contraction of a directly welded bar upon heating and cooling would produce undesirable stresses and the danger of brittle fracture of the intermetallic material together with disintegration of the weld interface. Obviation of these stresses is important since to be effective as an electrode, the composite bar must remain integral to insure a low electrical resistivity over a wide temperature range.

It is therefore an object of this invention to provide

5

2

for bonding particular refractory materials to a supporting metallic base and the composite article thereby produced.

It is still another object of this invention to provide such a bond wherein the desirable electrical properties are maintained.

It is a further object of this invention to provide a composite and integral electrode for electrolytic cells wherein the working end or tip only is formed of a refractory such as titanium diboride.

Still further objects and the entire scope of applicability of the present invention will become apparent from the detailed description given hereinafter; it should be understood, however, that the detailed description, while indicating preferred embodiments of the invention, is given by way of illustration only, since various changes and modifications within the spirit and scope of the invention will become apparent to those skilled in the art from this detailed description.

It has been found that the above objects may be attained by bonding the refractory article to a less expensive metallic base or shank by a novel method in which an alloy having desirable electrical resistivity and a coefficient of expansion compatible with that of the refractory material is utilized in forming the bond.

More particularly, the alloy is interposed between the refractory article and the metallic base and the members are bonded together with a special solder adapted to "wet" the refractory article. The bond is effected by heating the assembled article in a protective atmosphere to a temperature above the flow point of the solder but below the melting point of the members to be joined. The bonded assembly is then slowly cooled, the initial portion of the cooling cycle preferably conducted also in the protective atmosphere.

With reference to an embodiment of this invention relating to the production of a cathode, a refractory article, for example, in the form of a rod is inserted into an alloy cup into which has been placed the special solder. Beneath the alloy cup is placed the base of a metal of desired electrical resistivity, a portion of the same solder being used between the alloy cup and the metallic base. The assembled bar is placed in a furnace in a protective or an inert atmosphere, e.g., an atmosphere of an inert gas such as nitrogen, argon, hydrogen or helium, and heated to a temperature in excess of 1000° C. and preferably about 1100° C. This temperature is held for a time effective to insure complete flow of the solder, e.g., for about 10 minutes. The composite bar is then allowed to cool very slowly to insure against thermal breakage, 24 hours usually being sufficient. The protective atmosphere is maintained during the heating and soaking periods but it may be eliminated after the temperature drops below about 1000° in the cooling cycle.

The complete manufacture of such an electrode may be considered as broken down into two steps: first, that of providing the refractory tip which will project into the molten aluminum and second, that of joining the tip to a metallic base as outlined above. The refractory tip may be produced by standard powder metallurgy techniques including cold pressing and sintering or hot pressing. The tips mentioned in the detailed description below were prepared by hot pressing although articles produced by other techniques may be likewise treated.

An alloy which has been found to be particularly suitable for the purposes of this invention is a nickel-iron-cobalt alloy metal known commercially as "Kovar" by which name it will be referred to herein. The composition of this alloy is 29% nickel, 17% cobalt, about 0.2% manganese and the remainder iron. There are a

number of other alloys which might be employed in this invention but Kovar has been found to be especially suitable. The requirements placed upon the alloy are that it have an electrical resistivity in the general range of those of the intermetallic and metal utilized, that it have a coefficient of expansion compatible with that of the intermetallic and that it can be subjected to high temperatures. As set forth above, titanium diboride has a coefficient of expansion of  $8.1 \times 10^{-6}$  over the temperature range of 20° to 800° C., while iron or steel has an average value of about  $14 \times 10^{-6}$  over the temperature range of 20° to 700° C. Kovar alloy has an average coefficient of expansion of  $8.0 \times 10^{-6}$  over the temperature range of 20° to 700° C., almost identical to that of titanium diboride. The electrical resistivity of the Kovar alloy is also within the desired range, measuring 50 micro-ohm centimeters at room temperature, the values for titanium diboride and iron or steel being 15-25 and 10-20 micro-ohm centimeters respectively, also at room temperature. The function of the Kovar in the composite electrode is to prevent separation of the bond while providing a good path for the flow of current.

The solder which is utilized must allow for a low electrical resistivity, a high flow temperature, and provide an effective bond. One such solder contains a major proportion of silver and a minor proportion of manganese. The silver constituent provides the desired electrical properties and the manganese is important in that it will "wet" the refractory, while silver by itself will not. An alloy containing 85% silver and 15% manganese has a flow temperature of 950° C. and combines the wetting action of manganese with the desirable electrical properties of silver to produce an ideal bond.

Referring now to the drawing wherein like figures refer to like parts.

FIGURE 1 is a cross-sectional view of an assembly of a refractory article and a metallic base prepared according to one embodiment of this invention;

FIGURE 2 is a cross-sectional view of the assembly of FIGURE 1 after treatment according to this invention to form a composite and integral article; and

FIGURE 3 is a cross-sectional view of a composite and integral article prepared according to another embodiment of this invention.

The electrode shown in FIGURES 1 and 2 comprises a working end or tip 1 of titanium diboride placed within a cup 2 of Kovar. Beneath the Kovar cup is placed base 3 of iron or steel. Within the Kovar cup and also between the bottom of the cup and the base are placed thin shims 4 of silver alloy, several sheets being placed within the cup so that during flow of the molten solder, the void is completely filled. Prior to assembly, the parts to be bonded, namely the tip, the Kovar interfacial material and the iron or steel base are sand or shot blasted to roughen the surface and to remove any foreign matter, and further cleaned with organic solvents such as toluol, nethylene chloride or acetone. The shims of silver solder are in this embodiment cut into circles, the diameters of which match the parts to be joined, and are also cleaned with the solvent.

The bar assembled as in FIGURE 1 is placed in a furnace capable of being heated to a temperature of 200° C. in an hour and containing a protective or inert atmosphere. The firing temperature used in this embodiment was 1100° C., but this may vary depending upon the type of solder utilized and the density of the refractory material used in the tip. The bar was held at this temperature for 10 minutes insuring a good flow of the silver solder. The bar was then cooled over a time period of 24 hours, the inert atmosphere being unnecessary after the temperature fell below 1000° C. The completed composite and integral bar as shown in FIGURE 2 comprises the tip 1, Kovar cup 2 and base 3 bonded by the silver solder 5, now completely filling the voids between the

component parts and forming a strong bond therebetween.

A bar as formed in the above embodiment was tested in an experimental electrolytic cell built to simulate an actual aluminum production cell. Cycling between room temperature and 1000° C. did not disrupt the bond. After running steadily for two weeks in molten aluminum at 1000° C. and 12 days in molten cryolite at 1050° C., the average resistivity for the bar was the same as when the tests were first started. This indicates the high integrity of the bond. Also, the low average resistivity of 22 micro-ohm centimeters for the bar at room temperature about doubled at 1000° C. to 45 micro-ohm centimeters while carrying 100 amperes of current.

A second embodiment of this invention is illustrated in FIGURE 3 and is especially useful when bars of comparatively large diameter are produced. In this embodiment, in place of the Kovar cup 2, shown in FIGURES 1 and 2, a simple plate 6 of the Kovar alloy may be utilized. The base 7 is modified to provide a generally cup-shaped end portion 8. The Kovar plate 6 is placed within cup portion 8 already having silver solder in place at the bottom thereof. Additional solder is placed upon the Kovar plate. The end portion of refractory tip 9 which is inserted into cup portion 8 of base 7 is beveled slightly at 10 to correspond to the inner surface 11 of cup portion 8. After heating and cooling as outlined above, the solder has melted and flowed to fill the spaces 5 between the elements to form an integral bond therebetween.

The bars formed according to the preferred embodiments of this invention fulfill the requirements of cathodes to be used in electrolytic cells for the production of aluminum metal from alumina. The overall electrical resistivity of the bars is between 20 and 30 micro-ohm centimeters at room temperature. The bond formed is refractory, withstanding temperatures in excess of 800° C., and a bar when cycled from room temperature to 1000° C. in the cell maintains its integrity and therefore its low electrical resistivity. Moreover, this invention provides the additional advantage of a saving up to two-thirds of the cost of the intermetallic material normally needed in the production of a cathode.

What is claimed is:

1. A composite bar suitable for use as an electrode in an electrolytic cell comprising:

(1) a first member having low solubility in molten alumina said member being formed entirely from a material selected from the group consisting of titanium boride, titanium carbide, and zirconium boride;

(2) a metallic member selected from the group consisting of iron and steel and having a coefficient of expansion greater than that of said first member;

(3) a ferrous alloy member having a coefficient of expansion substantially equal to that of said first member and less than that of said metallic member interposed between said first member and said metallic member;

said members being bonded by a silver-manganese solder capable of wetting said first member.

2. The bar according to claim 1 wherein the solder comprises about 85% silver and about 15% manganese.

3. The bar according to claim 1 wherein the first member is titanium diboride.

#### References Cited in the file of this patent

#### UNITED STATES PATENTS

|           |          |               |
|-----------|----------|---------------|
| 1,524,218 | Smith    | Jan. 27, 1925 |
| 2,141,113 | Peterson | Dec. 20, 1938 |
| 2,439,570 | Hensel   | Apr. 13, 1948 |
| 2,708,787 | Chick    | May 24, 1955  |

#### FOREIGN PATENTS

|         |               |               |
|---------|---------------|---------------|
| 671,072 | Great Britain | Apr. 30, 1932 |
|---------|---------------|---------------|